

# UNITED STATES PATENT OFFICE.

ALFRED L. PELLEGRIN, OF TUCSON, ARIZONA, ASSIGNOR OF ONE-HALF TO HENRY GREENWELL, OF NOGALES, ARIZONA.

## PROCESS OF CONCENTRATING ORES.

1,237,691.

Specification of Letters Patent. Patented Aug. 21, 1917.

No Drawing. Application filed October 10, 1913, Serial No. 794,392. Renewed February 2, 1917. Serial No. 146,230.

*To all whom it may concern:*

Be it known that I, ALFRED L. PELLEGRIN, a citizen of the United States, residing at Tucson, in the county of Pima and State of Ariz., have invented a certain new and useful Improvement in Processes of Concentrating Ores, of which the following is a full, clear, and exact description, reference being had to the accompanying drawings.

- 10 This invention relates to a process of concentrating ores and has for its object the recovery of a larger amount of heavy or valuable minerals than is possible with the processes that are now generally practised.
- 15 As is well known, the present practice, especially in treating low grade copper ores and lead and zinc ores, is to crush wet; that is to say, with the admixture of a large proportion of water; such crushing being usually accomplished by means of stamps, after which the pulp is passed over jigs and concentration tables of various patterns. This crushing with a large proportion of water (whether the crushing is accomplished by 25 heavy stamps or by any of the various grinding mills) results in reducing a large amount of the valuable mineral being treated to an undesirable degree of fineness, rendering it extremely difficult, if not com- 30 mercially impossible, of recovery; this is especially so where the metallic minerals are much more soft and brittle than the gangue.

As is well known, when the ore is crushed dry (as by means of rolls or other dry 35 crushing machines) a much smaller proportion of fines is produced; in fact, when the dry crushing is properly conducted, the amount of any given size of the particular metallic mineral in the ore should bear the 40 same proportion to the gangue of that size that the entire amount of such mineral present in the ore bears to the entire amount of the gangue;—and the slimed minerals should not exceed this proportion to the slimed 45 gangue. However, as the process of ore concentration is usually practised (and principally because of the sliming action) in the best of the large mills now in operation the loss of values equals, and frequently exceeds, 30% of the total values contained in the original ore, and this loss is irretrievable.

In carrying out my invention, the ore is crushed dry, (by means of the usual crushers or rolls, or other dry crushing devices,) and

then separated into various predetermined sizes, reserving for special treatment the finest size—usually varying from 100 to 200 mesh. All sizes other than the aforesaid finest size are combined into two or more mixtures, the proportions of the various sizes in each mixture being different from the proportions in which these sizes existed in the crushed ore before separation into such sizes and the proportions of the sizes in one mixture being different from the proportions of the sizes in the other mixture. These mixtures thus formed are passed over or through dry jigs or concentration tables, whereby a certain proportion of the heavy minerals or values will be saved.—usually from 60 to 80%. After the ore has thus been passed once or twice through the dry concentrators, the values remaining, while difficult of recovery by any dry machine, are particularly amenable to treatment by any of the wet concentrating devices; and, if such ore be now admixed with the proper proportion of water and passed over a wet table or other concentrator, a practically perfect recovery of the contained values will result.

At the end of this operation, practically all of the values in the material treated will have been recovered, only the slimes (which should not amount to over 15% of the ore) being still untreated. These slimes will usually assay several times as much as the original ore and may be smelted, lixiviated, or reserved for treatment by some other process. Thus, instead of 30% or more of the value being irretrievably lost, practically none is lost,—a larger amount being directly saved in a marketable form and the rest stored for suitable treatment, and all at a less operating cost than is possible by the practice of processes heretofore practised.

A great advantage in combining the dry and wet processes in the manner indicated hereinbefore is that each seems to act better or more readily on certain sizes or conditions of the minerals than the other; and while the dry concentrates first obtained are of high grade, the wet concentrates next recovered are also of good grade, without re-treatment; thus the special advantages of each system are taken advantage of.

The slimes (of which only the very finest

2  
are reserved and which are impossible of concentration whether wet or dry and which interfere with the other sizes with which they may be combined) by the very reason 5 of their fineness are in the best possible condition for recovery by solution or by smelting after briquetting.

By the practice of my method, I have been able to realize repeatedly a saving of 92% 10 of the mineral present in the gangue, whereas, in the treatment of the same ores by methods heretofore in use, a recovery of 67% to 75% was the best that could be realized.

15 Having thus described my invention, what I claim is:—

1. The process of concentrating ore which consists in dry-crushing the ore, removing therefrom the finest sizes, forming the remaining sizes into mixtures containing varying sizes, subjecting such mixtures to dry concentration, and thereafter subjecting such mixtures to wet concentration.

2. The process of concentrating ore which 25 consists in dry-crushing the ore, removing therefrom the finest sizes, forming the remaining sizes into a mixture of varying sizes, subjecting such mixture to dry concentration, and thereafter subjecting such mixture to wet concentration.

3. The process of concentrating ore which 30 consists in dry-crushing the ore, separating the crushed ore into various predetermined sizes, combining all but the finest sizes into 35 two or more mixtures, subjecting such mix-

tures to dry concentration, thereafter subjecting the remaining values in such mixtures to wet concentration, and separately recovering the mineral from the finest sizes.

4. The process of concentrating ore which 40 consists in dry-crushing the ore, separating the same into various predetermined sizes, combining all but the finest sizes into two or more mixtures, the proportions of the sizes in each mixture differing from the proportions in which said sizes existed in the ore as crushed and before separating and the proportions of the sizes of one mixture differing from the proportions of the sizes in the other mixture, subjecting such mixtures to dry concentration, thereafter subjecting the mixtures to wet concentration, and separately recovering the mineral from the finest sizes.

5. The process of concentrating ore which 45 consists in dry-crushing the ore, separating the same into various predetermined sizes, mixing together the various sizes with the exception of the finest size, subjecting such mixture to dry concentration, thereafter subjecting the mixture to wet concentration, and separately recovering the mineral from the finest size.

In testimony whereof, I hereunto affix my signature in the presence of two witnesses. 55

ALFRED L. PELLEGRIN.

Witnesses:

GEO. P. MYERS,  
LUIS L. PELLEGRIN.